

1

3,707,413

ROCKET OXIDIZER COMPOSITION  
 Donald Pilipovich, Canoga Park, Calif., assignor to  
 North American Rockwell Corporation  
 No Drawing. Filed Apr. 3, 1968, Ser. No. 718,989  
 Int. Cl. C06b 15/00

U.S. CL. 149—109

2 Claims

## ABSTRACT OF THE DISCLOSURE

A liquid rocket oxidizer whose freezing point is below  $-65^{\circ}\text{F}$ . comprising  $\text{ClF}_3\text{O}$  and from 14 to 40 weight percent  $\text{ClF}_5$ .

## REFERENCES TO RELATED APPLICATIONS

This invention is related to copending U.S. application Ser. No. 543,493 and to U.S. Pat. No. 3,354,656.

## BACKGROUND OF THE INVENTION

The field of interhalogen chemistry has provided several promising new oxidizers. One of the areas of highest utility of these new oxidizers is in the field of rocket missile propulsion.

One of the newest of the interhalogen propellants is oxychlorine trifluoride,  $\text{ClF}_3\text{O}$ . It has great utility as a liquid rocket oxidizer due to its high specific impulse and density impulse. However,  $\text{ClF}_3\text{O}$  does have one disadvantage. Its freezing point is  $-37.2 \pm 0.5^{\circ}\text{C}$ . For tactical missile applications, it has been stated that it is necessary for the propellants to remain liquid at temperatures of at least  $-65^{\circ}\text{F}$ . ( $-54^{\circ}\text{C}$ ).

The addition of conventional freezing point depressants to  $\text{ClF}_3\text{O}$  would have the desired effect of lowering the freezing point. However, they would uniformly result in a deleterious effect to  $\text{ClF}_3\text{O}$ 's highly advantageous specific impulse and density impulse values.

It would be desirable to provide a freezing point depressant for  $\text{ClF}_3\text{O}$  that would not result in a reduction of more than about two percent of  $\text{ClF}_3\text{O}$ 's high density impulse.

It is an object of this invention to provide a means for depressing the freezing point of oxychlorine trifluoride,  $\text{ClF}_3\text{O}$ .

It is a further object of this invention to reduce the freezing point of  $\text{ClF}_3\text{O}$  to below  $-65^{\circ}\text{F}$ .

It is a still further object of this invention to reduce the freezing point of  $\text{ClF}_3\text{O}$  to below  $-65^{\circ}\text{F}$ . without reducing the density impulse of the resulting oxidizer to less than 98 percent of that of pure  $\text{ClF}_3\text{O}$ .

It is a still further object of this invention to reduce the freezing point of  $\text{ClF}_3\text{O}$  to below  $-65^{\circ}\text{F}$ . without substantially changing its properties of specific impulse and density impulse.

Further objects and advantages of this invention will become apparent from the following description.

## DESCRIPTION OF THE INVENTION

It has been found that the addition of at least 14 weight percent of  $\text{ClF}_5$  to  $\text{ClF}_3\text{O}$  results in the depression of freezing point of the mixture to below  $-65^{\circ}\text{F}$ .

It has been further found that the addition of up to 40 weight percent of  $\text{ClF}_5$  results in a reduction in density impulse of  $\text{ClF}_3\text{O}$  of typically less than two percent. Further, there is only a very minor effect on specific impulse. This effect can be advantageous, that is, an increase in specific impulse can be observed.

It has been unexpectedly found that a mixture of  $\text{ClF}_5$  and  $\text{ClF}_3\text{O}$  according to the teachings of this invention results in a maximum specific impulse point for fuels containing carbon or boron. Examples of such fuels are monomethylhydrazine and diborane. Further, this maximum

2

can occur within the 14–40 weight percent range recited above. Usually it occurs between 15–25 weight percent  $\text{ClF}_5$ .

With monomethylhydrazine a maximum specific impulse occurs at about 70 percent  $\text{ClF}_3\text{O}$  and 30 weight percent  $\text{ClF}_5$ . In the case of the fuel MHF-3 which is a 85/15 mixture of monomethylhydrazine and hydrazine, a maximum occurs at about 65 weight percent  $\text{ClF}_3\text{O}$  and 35 weight percent  $\text{ClF}_5$ .

While not wishing to be bound by theory, it is believed that these maxima occur at the point where stoichiometric ratio of one oxygen atom is supplied for every carbon or boron atom in the fuel. If less oxygen than this is supplied, either free carbon or  $\text{CF}_4$  is produced, depending on the oxidizer to fuel mixture ratio. If more oxygen than this is used, the compound carbon dioxide is formed. As will be clear to those skilled in the art, the compound CO is the most desirable reaction product, since it has the lowest molecular weight of all the possible carbon containing gaseous products.

Naturally the oxidizer combination of the instant invention is not limited to use with fuels containing carbon or boron such as the two examples given above. The oxidizer combination is also suitable for use with fuel such as hydrogen, hydrazine and metallized liquids. However, it is only with those fuels containing carbon or boron that a maximum in specific impulse is noted at a stoichiometric ratio of oxygen in the oxidizer to carbon in the fuel of about 1:1.

The following examples illustrate the novel oxidizers of this case.

## EXAMPLE I

A mixture of 15 weight percent  $\text{ClF}_5$  in  $\text{ClF}_3\text{O}$  is made. A freezing point determination showed a freezing point of  $-55^{\circ}\text{C}$ . This oxidizer gave the specific impulse of 301 sec. when tested with the fuel MHF-3 and a density impulse of 445.6 gram-sec./cc. Pure  $\text{ClF}_3\text{O}$  froze at  $-38^{\circ}\text{C}$ . and gave a specific impulse of 299 sec. and a density impulse of 445 gram-sec./cc.

## EXAMPLE II

39 weight percent  $\text{ClF}_5$  in  $\text{ClF}_3\text{O}$  was found to have a freezing point of  $-90^{\circ}\text{C}$ . When tested with MMH it was found to have a specific impulse of 299.8 sec. and a density impulse of 439 gram-sec./cc. Pure  $\text{ClF}_3\text{O}$  with MMH had a specific impulse of 298.1 sec. and a density impulse of 443 gram-sec./cc.

It is to be understood that the above described embodiments are merely illustrative of application of the principles of this invention. Those skilled in the art may readily devise other variations that will embody the principles of the invention. It is, therefore, to be understood that within the scope of the appended claims the invention may be practiced otherwise than as specifically described.

What is claimed is:

1. A rocket oxidizer composition consisting essentially of  $\text{ClF}_3\text{O}$  and from 14 to 40 weight percent  $\text{ClF}_5$ .
2. The rocket oxidizer of claim 1 wherein the  $\text{ClF}_5$  comprises from 15 to 25 weight percent of the mixture.

## References Cited

## UNITED STATES PATENTS

- |           |         |                       |         |
|-----------|---------|-----------------------|---------|
| 3,170,282 | 2/1965  | Kirshenbaum et al. -- | 149—1 X |
| 3,260,628 | 7/1966  | Logan et al. -----    | 149—1   |
| 3,354,646 | 11/1967 | Maya et al. -----     | 149—1 X |
| 3,377,801 | 4/1968  | Altman -----          | 149—1 X |

BENJAMIN R. PADGETT, Primary Examiner

70 S. J. LECHERT, Jr., Assistant Examiner

U.S. CL. X.R.

149—1, 22, 36